

## UNITED STATES PATENT OFFICE

2,030,892

## MATCH MANUFACTURING

Michail G. Pelipetz, New York, N. Y., assignor of  
one-half to Peter L. Doodchenko, New York,  
N. Y.

No Drawing. Refiled for abandoned application  
Serial No. 585,242, January 7, 1932. This ap-  
plication February 8, 1935, Serial No. 5,617

3 Claims. (Cl. 52—25)

This case is a substitute for abandoned applica-  
tion 585,242 filed January 7, 1932.

My invention relates to match manufacturing  
and has particular reference to the manufacture  
5 of striking composition for match containers.

The match boxes or books for the use with  
safety matches are usually provided with a coating  
of striking composition containing phosphorus  
and some friction or abrasive material. This  
10 material is prepared as paste with glue and water  
and is applied in a semi-liquid form.

All these compositions have a serious disadvan-  
tage that they are affected by water and moisture  
which softens the glue base and renders impos-  
15 sible to generate sufficient friction for igniting  
the matches. Another disadvantage of these com-  
positions is that they require special drying process  
during the manufacture of boxes and books,  
causing additional expense for fuel. Vapors and  
20 fumes generated during this drying process are  
injurious to the health of workmen and require  
additional and expensive ventilating system.

In order to eliminate these objections I provide  
a composition with substances insoluble in water  
25 which are liquefied by melting them in a special  
container and applied to the paper of the boxes  
and books while still hot. The striking powder  
is sprayed over the coating while the latter is  
still soft.

For this purpose I use a binder representing a  
30 mixture of several ingredients having different  
viscosities and melting points, thereby controlling  
the desired final viscosity of the melted mixture  
and its melting temperature. I have found that  
35 good results are obtained with a mixture of resinous  
substances which can be melted at a suffi-  
ciently low temperature and which become solidified  
and hard at the room temperature.

By combining resinous, tarry and similar sub-  
40 stances in various proportions in accordance with  
their individual properties, I obtain a composi-  
tion with the following requisite properties:

1. Melting temperature of about 80° or 90° C.,  
45 or just below the boiling point of water. Such  
a temperature prevents the excessive drying of  
paper during the process of formation of the  
striking layer and, at the same time, it is suffi-  
ciently high so that the coating remains hard  
at all ordinary temperatures.

50 2. The composition must be sufficiently hard  
at ordinary temperatures in order to retain firmly  
in the striking powder.

3. The composition must be sufficiently elastic  
so as not to break when the paper is slightly bent.

55 4. The composition must be insoluble in water

so as to render the striking coating waterproof,  
the striking powder being also unaffected by  
water.

5. The composition must have sufficient vis-  
cosity when melted in order to flow freely over  
the paper and to penetrate it to a certain extent  
in order to adhere firmly to the surface of the  
paper. This viscosity must correspond to the de-  
gree of porosity of the paper, lower viscosity being  
required for harder grades of paper.

I have found that rosin obtained by distilla-  
tion of the raw turpentine or pitch represents the  
most suitable basic material or ingredient for my  
composition. In order to increase its hardness  
I add a small quantity of shellac.

15 The melting point of rosin and shellac being  
somewhat too high, I lower it by adding raw  
turpentine or turpentine pitch.

I have found that asphalt and similar tarry  
substances, pitch etc., can be added to rosin, in-  
creasing its hardness at ordinary temperatures.

The above materials form a first group of in-  
gredients, characterized by the higher melting  
point and hardness at ordinary temperatures,  
25 with sufficient viscosity when melted. They are  
somewhat brittle, however, when cold, and to  
increase the elasticity of the composition at or-  
dinary temperatures I add ingredients of the sec-  
ond group which also tend to lower the melting  
30 temperature. This group includes such materials  
as waxes, paraffin, stearin, turpentine oil, and  
similar substances.

In general, I use a mixture of aliphatic and  
aromatic hydrocarbons and their derivatives, in-  
35 soluble in water, with melting temperature not  
over 150° C., the melting point of the composi-  
tion being preferably about 80° or 90° C. Mate-  
rials of the second group may be even liquid at  
ordinary temperatures, for instance, turpentine  
40 oil. Materials of the first group must be in col-  
loidal form.

The following example represents a composi-  
tion with melting point of about 90° C. and is  
otherwise suitable for paper of ordinary density.

*Example I*

|                  | Per cent by weight |
|------------------|--------------------|
| Rosin            | 95                 |
| Turpentine pitch | 3                  |
| Shellac          | 1                  |
| Paraffin         | 1                  |

Paraffin may be replaced by stearin, wax or  
similar material.

Gutta percha can be also added to the composition, increasing its viscosity, as per Example II.

*Example II*

|              | Per cent by weight |
|--------------|--------------------|
| 5 Rosin      | 85                 |
| Gutta percha | 10                 |
| Shellac      | 3                  |
| Paraffin     | 1                  |
| 10 Wax       | 1                  |

15 Gutta percha lowers the melting point so that a larger amount of shellac may be added. Its greater hardness and brittleness require addition of a larger percentage of paraffin and wax. Paraffin or stearin alone should not be added in a large quantity as these substances render the composition oily and less adherent to the paper.

20 These composition retain viscosity until fully hardened. The striking powder must be sprayed over the composition on the paper at a somewhat reduced temperature, when the composition begins to thicken but still retains its adhesive properties to catch and hold the powder. Usually a drop of from 10 to 30° C. is required for this purpose, so that if a temperature of 90° C. is maintained in the melting pot, then a temperature of about 60° to 70° C. must be maintained at the drum.

25 My method has important advantages over ordinary methods using water soluble glue, as follows:

30 1. My striking coating on match containers is fully waterproof.  
35 2. The smallest possible amount of striking powder is used, as it is applied to the surface of the coating only, and all the excess powder is collected and used over again.

With water soluble compositions the striking powder is mixed with glue and gradually settles 40 down during the process. The mixture therefore becomes poorer and poorer in certain ingredients which settle more rapidly, necessitating frequent discarding of such residue.

3. With water solutions large and expensive driers are required, which consume a large amount of heat. This heat is largely wasted through radiation and ventilation.

4. Expensive ventilating system is required 5 with water solutions, which is not needed with my system.

5. The absence of noxious vapors in my process tends to render it more hygienic.

6. Paper in the wet process becomes stretched 10 and weakened, and often breaks causing expensive stoppages in the process. With my process the paper is dry and it retains its strength during the process.

7. With my process the paper comes out from 15 the machine ready for use, and the process is shortened very considerably.

8. A much smaller floor space is required for my process.

9. All danger is largely eliminated with my 20 process, as boxes or books containing matches are not required to be placed in driers at an increased temperature.

I claim as my invention:

1. A striking composition for match boxes, consisting of from 85% to 95% of rosin by weight, from 1% to 3% of shellac, from 1% to 2% of paraffin and wax, and from 3% to 10% of resinous material taken from a group consisting of turpentine, pitch, and gutta percha, said ingredients 30 forming a binder, and a ground abrasive material imbedded in said binder.

2. A striking composition for match containers, consisting of rosin with small addition of shellac, paraffin and wax, mixed at the surface with a 35 ground abrasive material.

3. A striking composition for match containers, consisting of resinous and tarry substances with a small addition of shellac, paraffin and wax, mixed with a ground abrasive material. 40

MICHAIL G. PELIPETZ.